

June 4, 1935.

T. H. WARNER

2,003,524

## ALLOY

Original Filed Aug. 27, 1931



INVENTOR  
Thomas H. Warner  
BY  
Gustav R. Thompson  
ATTORNEY

## UNITED STATES PATENT OFFICE

2,003,524

## ALLOY

Thomas H. Warner, Union City, N. J., assignor to  
Metal Alloys, Inc., Wilmington, Del., a corpora-  
tion of Delaware

Application August 27, 1931, Serial No. 559,696  
Renewed November 1, 1934

2 Claims. (Cl. 75—1)

This invention relates to light metal alloys having an aluminum or magnesium base, and provides improvements therein.

Industry is greatly interested in light metal alloys for structural use,—notably in connection with air-craft, motors, etc. For structural use the light alloys "duralumin" and "magnalium" are probably the most satisfactory at present used. There remains nevertheless a want for a light metal alloy or alloys possessing better mechanical or physical properties than possessed by those now on the market, notably better tensile strength and greater resistance to "fatigue"; and better chemical properties, notably greater resistance to corrosion.

The present invention provides improved light metal alloys having greater tensile strength, greater resistance to "fatigue", and greater resistance to corrosion compared with duralumin and magnalium, and which are tough, ductile and machineable. Alloys of the present invention further possess a good electrical conductivity.

Alloys according to the present invention have an aluminum or magnesium base and contain boron, vanadium, zinc, some magnesium when aluminum is the base and some aluminum when magnesium is the base, the range thereof in the alloys being approximately in percent by weight as follows:

|           | Aluminum base | Percent     |
|-----------|---------------|-------------|
| Boron     |               | 0.25 to 1.5 |
| Magnesium |               | 0.5 to 1.5  |
| Vanadium  |               | 0.25 to 1.  |
| Zinc      |               | 1. to 4.    |
| Aluminum  |               | 98. to 92.  |

|           | Magnesium base | Percent     |
|-----------|----------------|-------------|
| Boron     |                | 0.25 to 1.5 |
| Aluminum  |                | 0.5 to 1.5  |
| Vanadium  |                | 0.25 to 1.  |
| Zinc      |                | 1. to 4.    |
| Magnesium |                | 98. to 92.  |

The herein described improved alloys have been produced by placing the constituent metals together in an electric crucible furnace and melting under a vacuum. The apparatus used is illustrated diagrammatically in vertical section in the accompanying drawing, wherein numeral 10 designates a crucible of cast iron lined with alumina as indicated at 11, sealed with a vacuum

tight cover 12. Numeral 14 designates a vacuum-pump connected to the interior of the crucible preferably through a tank 15. Numeral 16 designates heating coils or windings around and beneath crucible 10 connected to a supply 18 of electric current. Numeral 20 designates a mold in which the alloy may be cast. The mold 20 is contained in a closed chamber 22 which is connected to vacuum pump 14 through tank 15.

The metals of which the alloys are composed, as set forth above, and within the ranges set forth above, are introduced into the crucible 10, with the metal constituting the base surrounding the other metals. The cover 12 is sealed onto the crucible, and a high vacuum produced in the interiors of the crucible and chamber 22, an equilibrium of vacuum being maintained during heating in chamber 22 and crucible 10. Electric current in the coils 16 heats the crucible and the metals contained therein. Fusion is effected at 20 a temperature of approximately 700°—800° Centigrade, this temperature being maintained for about 30 minutes for a  $\frac{1}{2}$  pound charge.

After the fusion has been completed as aforesaid and while a high vacuum is maintained in chamber 22, the melt is run into the mold 20 whereupon the alloy is solidified or formed into an ingot or casting by the chill of the mold. For running the melt into mold 20 a siphon tube 24, passing through the bottom of crucible 10 into the top of chamber 22 above mold 20, may be provided. By manipulating cocks 27, 28 in the lines from the vacuum tank 15, to crucible 10 and chamber 22 respectively, the pressure in crucible 10 may be raised (by admitting air thereto) while the vacuum is maintained in chamber 22, which results in the molten alloy in crucible 10 being siphoned through tube 24 into mold 20. For preventing "freezing" or solidification of the alloy in tube 24, an electrical resistance heater 30 surrounding tube 24, may be provided. The cast metal is allowed to stand in the mold under vacuum until the temperature falls to a suitable or desired degree, whereupon air may be admitted and the cooling accelerated. After cooling, the cast alloy is preferably aged by either immersing in hot oil or by other suitable and well-known methods.

The alloys hereinbefore described are light, dense, tough, ductile, possess great tensile

strength, are highly conductive electrically and are highly resistant to corrosion. For example, tests on an "aged" alloy (produced as hereinbefore described), having the specific composition

|             | Percent |
|-------------|---------|
| Boron       | .75     |
| Vanadium    | .25     |
| Magnesium   | 1.      |
| Zinc        | 1.      |
| 10 Aluminum | 97.     |

show that it has a tensile strength of 35,000 to 40,000 pounds per square inch, is tough, ductile, malleable and machineable, and after immersion 15 in five percent sulphuric acid for one week showed no visible attack when examined under a micro-

scope, and has a specific gravity of about 2.8.

What is claimed is:

1. An alloy of aluminum, magnesium, boron, vanadium and zinc (aluminum being the base) within the following ranges:

|             | Percent    |
|-------------|------------|
| Boron       | .25 to 1.5 |
| Magnesium   | .5 to 1.5  |
| Vanadium    | .25 to 1.  |
| Zinc        | 1. to 4.   |
| 10 Aluminum | 98. to 92. |

2. An alloy containing substantially three-fourths percent boron, one-quarter percent vanadium, one percent magnesium, one percent zinc and ninety-seven percent aluminum.

THOMAS H. WARNER.